

1

3,255,012

**SENSITIZED COLOR PHOTOGRAPHIC EMULSIONS  
AND PROCESSES CONTAINING COLOR COUPLERS**

Hans Glockner, Pullach, near Munich, Fritz Muller, Munich-Pasing, and Hugo Zorn, Lochhausen, near Munich, Germany, assignors to Agfa Aktiengesellschaft, Leverkusen-Bayerwerk, Germany, a corporation of Germany

No Drawing. Filed Aug. 23, 1965, Ser. No. 481,892  
Claims priority, application Germany, Aug. 20, 1960,

P 25,553

9 Claims. (Cl. 96—100)

This application is a continuation-in-part application of copending United States application Serial No. 131,929, filed August 16, 1961.

This invention concerns improvements in or relating to color photographic emulsions and processes.

More particularly it relates to the preparation of color-responsive silver halide emulsions suitable for use in the production of single- or more usually multi-layer color photographic media, which upon exposure and development in the appropriate manner will yield either a negative or positive color image, according to principles and techniques in themselves now well known.

In the preparation of color-responsive silver halide emulsions it is conventional to incorporate in the emulsion destined to form any given layer not only silver halide and a so-called sensitizer capable of enhancing the photo-sensitiveness of the silver halide to those wavelengths of light to which that layer is intended to respond, but also a so-called color coupler whose function is to react with the oxidation product of the developer to form a dye of the appropriate color. Where multi-layer color photographic media are intended to be built up by superimposing differently sensitized layers upon a film base or other support it is obviously necessary to ensure that the color couplers incorporated in any one layer do not diffuse or otherwise migrate into the adjacent layer or layers.

Two fundamentally different approaches have hitherto been adopted therefore in the preparation of color-responsive silver halide emulsions intended primarily for the production of multi-layer photographic media, but which it will of course be understood may equally serve for the production of single layers.

In one approach to the problem of securing a sensitized silver halide emulsion containing a diffusion-resistant color coupler, which for convenience will hereinafter be referred to as "process I" and which is typified by color film sold under the name "Agfacolor," the compounds employed as the color couplers are soluble in water, achieved by the substitution of sulpho- or carboxyl-groups into the molecule, but their diffusion resistance is ensured by the presence of a long aliphatic hydrocarbon chain in the molecule, as described for instance in German Patent 726,611. In the preparation of the emulsion these water-soluble compounds are merely dissolved in dilute sodium hydroxide solution and thereupon added to and thoroughly mixed with the silver halide emulsion.

The other approach to the problem, which for convenience will hereinafter be referred to as "process II" and which is typified by color film sold under the name "Ektachrome," involves the use as color couplers of compounds which are insoluble in water. In order to incorporate these water-insoluble color couplers in the silver halide emulsion it is however necessary to proceed in the manner which has been described in United States Patent 2,322,027, according to which the color coupler is first made up into a solution with a so-called oil former, usually a high-boiling point solvent insoluble in water, and this oily solution is then dispersed in droplets through-

2

out an aqueous gelatin solution, and finally the dispersion thus prepared is mixed with the silver halide emulsion. In this process the need for inherent diffusion-resistance of the color couplers themselves is greatly reduced, since their water-insolubility and their dispersion in conjunction with the oil former combine to impart a measure of protection against diffusion.

With both of these known types of process it is of course quite possible to achieve satisfactory results, but nevertheless both process I and process II have their disadvantages. In process I these stem primarily from the surface active effects of the color couplers, which are soap-like in character and consequently exert a strong influence upon the viscosity of the prepared emulsion, giving rise to difficulties during the coating procedure. In process II the disadvantages are attendant upon the use of oil-formers, whose presence in the form of distribution of oily droplets lends an undesired moistness to the finished emulsion-layer and can moreover give rise to color fogging during the development process.

Attempts have been made to find a process which avoids the disadvantages both of process I, due to the presence of solubilizing groups in the coupler molecule, and also those of process II, due to the use of an oil former. Color couplers have in fact already been described, in for example German Patent 725,872, which as a result of the presence of a long aliphatic hydrocarbon chain are diffusion-resistant, and which, since they contain no sulpho- or carboxyl-groups, are practically insoluble in water. It is moreover feasible to produce fine dispersions of such color couplers without the use of an oil former by dissolving them in a low-boiling point water-immiscible solvent and dispersing this solution with the aid of a wetting agent in an aqueous gelatin solution. The low-boiling point solvent can then be removed immediately, for example by evaporation, or removal can take place subsequently, after mixing of the dispersion with the silver halide emulsion, upon drying of the finished layer of emulsion formed in the coating procedure. Development of such a finished layer with a conventional color developer gives a clear and intense color image; but unfortunately other unexpected difficulties arise when an attempt is made to build up photographic media on the basis of emulsions containing such coupler dispersions, inasmuch as the usual sensitizers employed in such emulsions have been found to be incompatible in the silver halide emulsion with coupler dispersions of this kind.

It has in fact been established that the majority of the dyes hitherto proposed for use as photo-sensitizers for silver halide are unsuitable for use in conjunction with this kind of coupler dispersion. Their unsuitability demonstrates itself in practice in terms of a decline from hour to hour of the spectral sensitivity of such an emulsion upon standing. As a result a coating procedure of long duration, and even exceeding several seconds, becomes impractical, and moreover a generally similar decline in the spectral sensitivity is encountered upon storage of the finished layer. This rather surprising state of affairs can presumably be accounted for by the hypothesis that in this process the sensitizer is displaced from the silver halide surface by the color coupler whereas in processes I and II, respectively, the water-solubility of the coupler in the one case and the presence of the oil former in the other case prevent the coupler from competing with the sensitizer for adsorption onto the silver halide grains.

It is an object of the present invention to provide color photographic emulsions and processes which largely or wholly avoid the disadvantages of all these known procedures, and this is achieved by a careful selection of certain types of color coupler for use with certain types of sensitizer.

It has in fact now been found:

(1) That for the production of the cyan image it is possible to use phenolic color couplers whose molecule contains a long carbon chain with from 10 to 21 carbon atoms but no acid groups, since these in the absence of an oil former are fully compatible in a silver halide emulsion with red sensitizers provided that the latter are chosen from the class of *ms*-alkyl-benzthio- or -benzseleno-carbocyanines whose two ring nitrogen atoms are substituted by carboxy-alkyl groups.

(2) That for the production of the magenta image it is possible to use pyrazolone color couplers whose molecule contains a long carbon chain with from 10 to 21 carbon atoms but no acid groups, since these in the absence of an oil former are fully compatible in a silver halide emulsion with green sensitizers provided that the latter are chosen from the class of benzthio- or -benzseleno-pseudocyanines in which one ring nitrogen atom is substituted by a carboxyl-alkyl group.

Using these combinations of a type of coupler known per se with a type of sensitizer known per se, stable emulsions can be prepared from which single- or multi-layer color photographic media can be built up, and since no acid groups are present in the coupler molecule and the use of oil formers is unnecessary the previously-explained disadvantages of both processes I and II are avoided. The procedure used according to this invention in fact gives highly satisfactory results contrary to expectation in the light of knowledge about the liability for a decline of spectral sensitivity in the absence of an oil former and surprising insofar as they were not predictable from the individual properties of the respective selected classes of coupler and sensitizer. Emulsions prepared in accordance with this invention are easy and safe to handle during the coating operation, and the layers formed from them do not display the disadvantages which are observed upon use of oil formers. In particular the total volume of the finished emulsion is somewhat reduced and the dye image ultimately formed is highly stable, while the finished layer displays an outstanding resistance to abrasion or other mechanical damage as compared with the known layers containing oil formers.

The dyes which are used as the sensitizers according to the invention have the following general formula:

#### RED SENSITIZERS



#### GREEN SENSITIZERS



In the two general formulas shown above Y represents sulphur or selenium, R represents an alkyl group, A represents an alkylene group, one R<sub>1</sub> is a lower alkyl radical and the other R<sub>1</sub> —A—COOH and X represents an anion, while the benzene nucleus can bear any of the usual substituents, such as alkyl, alkoxy, naphthyl groups, halogen atoms and so on. The most diverse anions may be employed, including inter alia the following, namely halogen anions such as chloride, bromide and iodine, also perchlorate, sulphate, monoalkylsulphate, acetate and the like. Instead of the salt form

shown these dyes can in fact also be employed in the form of the corresponding betaine.

It will be observed that all the sensitizers to be used according to this invention have as a common characteristic a carboxy-alkyl group in the molecule. Dyes possessing this characteristic are in fact already known, having been described for example in German Patent No. 704,141 and indeed they are known to be suitable for use in conjunction with color couplers in silver halide emulsions. Whereas however it is possible, using these sensitizers or indeed many others to produce stable combinations of sensitizer—color coupler—silver halide when the procedures of the aforesaid processes I or II are employed, with of course the attendant disadvantages which have been previously described, what has hitherto never been recognized is that only by the selection of these sensitizers characterized by the presence of the carboxy-alkyl substituent, for use in conjunction with the classes of color coupler selected in accordance with this invention, does it become possible to achieve, in the absence of an oil former, results which in general are satisfactory and in particular are free from the disadvantages previously specified herein.

Color couplers suitable for forming the cyan or blue-green image according to the invention are derivatives of phenol or  $\alpha$ -naphthol having a long aliphatic hydrocarbon residue in the molecule. The carbon chain should be sufficiently long in order to arrest diffusion completely, and to this end in general a chain length of over 10 carbon atoms is needed: the optimum chain length in any particular circumstances can easily be determined by tests. In most cases the preferred couplers are those in which the chain consists of 17 or 18 carbon atoms. Such phenol or  $\alpha$ -naphthol derivatives per se are known, as well as methods of preparing them, and need not be further described herein. It should be noted that, provided the carbon chain contains from 10 to 21 carbon atoms, it is immaterial whether it is straight- or branched-chain and it may be an unsubstituted hydrocarbon chain or if desired can bear any of the usual substituents, such as aryl, alkoxy- or aryloxy- groups.

Merely by way of illustration the following compounds are listed as examples of cyan color couplers suitable for use in accordance with the present invention:

- 45 5-stearoylamino-1-naphthol
- 1-hydroxy-2-naphthoic acid (4'-octadecyloxy)-anilide
- N,N'-dodecamethylene-bis-(1-hydroxy-2-naphthyl-amide)
- 50 1-hydroxy-2-naphthoic acid octadecylamide
- 1-hydroxy-4-bromo-naphthoic acid octadecylamide
- 1-hydroxy-4-chloronaphthoic acid octadecylamide
- 1-hydroxy-4-bromo-naphthoic acid hexadecylamide
- 1-hydroxy-4-chloro-naphthoic acid hexadecylamide
- 55 1-hydroxy-2-naphthoic acid N-octadecyl-anilide
- 1-hydroxy-2-naphthoic acid dodecyloxy-butylamide
- 2,4-dichloro-5-stearoylamino-1-naphthol
- 2-palmitoylamino-4-chloro-5-methyl-phenol
- 2-octadecyl-4-chloro-phenol

As regards the pyrazolone color couplers to be used according to the present invention for forming the magenta image the same remarks concerning the length and nature of the aliphatic chain hold good as in the case of those employed to form the cyan image. Again, merely as illustration, the following compounds are listed as examples of suitable magenta color couplers:

- 1-phenyl-3-heptadecyl-pyrazolone-5
- 1-phenyl-3-stearoylamino-pyrazolone-5
- 70 1-(2'-benzthiazolyl)-3-dodecyl-pyrazolone-5
- 1-phenyl-3-pentadecyl-pyrazolone-5
- 1-(2'-aminophenyl)-3-heptadecyl-pyrazolone-5
- 1-(4'-bromophenyl)-3-pentadecyl-pyrazolone-5
- 75 1-(2',4'-dichlorophenyl)-3-heneicosyl-pyrazolone-5

1-(2',4',6'-trichlorophenyl)-3-stearoylaminopyrazolone-5  
 1-(2',4',6'-trichlorophenyl)-3-heptadecylamino-  
 pyrazolone-5

The dispersion of the color coupler must not be effected with the aid of oil formers such as those which are used, for example, in the process of U.S. Patents 2,304,940 and 2,322,027 because they have the disadvantages mentioned above in the specification.

The dispersion of the color coupler is instead effected according to methods well known to those skilled in the art in order to distribute water-insoluble substances as finely as possible in aqueous media. Thus, for instance, the color couplers may be dispersed in low boiling point, water immiscible solvents such as ethyl acetate, propyl acetate, methyl propionate, chloroform, nitroethane, nitromethane and the like, which are removed again from the emulsion in the course of the process.

However, the desired dispersions may also be obtained by finely milling the coupler substances in a colloid mill.

Another method for effecting the dispersion consists of stirring the couplers in the presence of a strong alkali and of a known wetting agent with the gelatin solution, whereupon the gelatin solution is subsequently neutralized by the addition of an acid. In all instances a very fine dispersion is obtained which dries completely transparent after pouring it onto a photographic film carrier.

The red-sensitizers which are to be used according to the invention in combination with the specified phenolic cyan couplers should possess a narrowly limited spectral sensitization band at the red end of the spectrum, and this requirement is apparently best achieved by choosing ethyl residue as the alkyl substituent in the *m*-position (see the above general formula). While other carboxy-alkyl groups are suitable as the nitrogen substituent a  $\beta$ -carboxy-ethyl group is preferably employed. Illustrative examples of suitable red sensitizer dyes are shown in the following list:

- 1,1-di-( $\beta$ -carboxy-ethyl)-5,6,5',6'-tetramethyl-9-ethyl-benzthio-carbocyanine iodide
- 1,1'-di-( $\beta$ -carboxy-ethyl)-6,6'-dichloro-9-ethyl-benzthio-carbocyanine iodide
- 1,1'-di-( $\beta$ -carboxy-ethyl)-6,6'-dimethoxy-9-ethyl-benzthio-carbocyanine iodide
- 1,1'-di-( $\gamma$ -carboxy-propyl)-5,6,5',6'-tetramethyl-9-ethyl-benzthio-carbocyanine iodide
- 1,1'-di-( $\gamma$ -carboxy-propyl)-6,6'-dichloro-9-ethyl-benzseleno-carbocyanine iodide
- 1,1'-di-( $\gamma$ -carboxy-propyl)-6,6'-dimethoxy-9-ethyl-benzthio-carbocyanine bromide
- 1,1'-di-( $\gamma$ -carboxy-ethyl)-5,5'-dimethoxy-6,6'-dimethyl-9-ethylbenzthio-carbocyanine iodide
- 1,1'-di-( $\beta$ -carboxyethyl)-6,6'-dichloro-9-ethyl-benzseleno-carboxycyanine iodide

The green-sensitizers which are to be used according to the invention in combination with the specified pyrazolone magenta couplers may for example include the following:

- 1-( $\beta$ -carboxy-ethyl)-1'-ethyl-6,6'-dimethoxy-benzseleno-pseudocyanine iodide
- 1-( $\beta$ -carboxy-ethyl)-1'-ethyl-6-phenyl-6'-methoxy-benzthio-pseudocyanine bromide
- 1-( $\beta$ -carboxy-ethyl)-1'-ethyl-5-methyl-6,6'-dimethoxy-benzseleno-pseudocyanine iodide
- 1-( $\beta$ -carboxy-ethyl)-1'-ethyl-4,5-naphtho-pseudocyanine bromide

It will of course be understood that, as regards the sensitization effect, it is in every respect a matter of indifference whether the dye salt or the corresponding betaine is employed, and that, as regards the dyes themselves, these may be obtained in accordance with known methods.

In order that the invention may be well understood the following illustrative examples will now be given:

Example 1.—Production of a silver halide emulsion for the cyan image

1 kg. of a silver bromide emulsion prepared in the usual way is sensitized with 30 mg. of 1,1'-di-( $\beta$ -carboxy-ethyl)-6,6'-dimethoxy-9-ethyl-benzthio-carbocyanine, dissolved in ethanol.

A coupler dispersion is then introduced, which is prepared in the following manner: 10 g. of 1-hydroxy-2-naphthoic acid octadecylamide are dissolved in 30 ml. of ethyl acetate with warming, and dispersed in a colloid mill with 160 ml. of 5% gelatin solution which contains 1 g. of dodecylbenzene-sulphonate. The ethyl acetate is then removed from this dispersion by evaporation.

After the mixing of the coupler dispersion with the silver halide emulsion, and introduction of the conventional coating additives the finished emulsion is coated onto a film base in the usual manner and dried.

After exposure through a grey-wedge behind a red filter, development in a dialkyl phenylenediamine developer and bleaching of the silver, an intense clear blue-green wedge is obtained. The same sensitometric data are secured if the finished emulsion has been allowed to stand for several hours before the coating operation. Moreover if the finished layer is subjected to an accelerated storability test, no decline in sensitivity is observed, or at most only a quite insignificant decline.

Substantially similar results may be secured by substituting any of the following couplers, namely 1-hydroxy-4-chloro-naphthoic acid octadecylamide, 1-hydroxy-2-naphthoic acid N-octadecyl-anilide, 1-hydroxy-2-naphthoic acid dodecyloxy-butylamine and 1-hydroxy-2-naphthoic acid octadecylamide, and/or any of the following sensitizers, namely 1,1'-di-( $\beta$ -carboxy-ethyl)-6,6'-di-chloro-9-ethyl-benzseleno-carbocyanine iodide, 1,1'-di-( $\beta$ -carboxy-ethyl)-5,5'-dimethoxy-9-ethyl-benzthio-carbocyanine iodide, 1,1'-di-( $\beta$ -carboxy-ethyl)-6,6'-dichloro-9-ethyl-benzthio-carbo-cyanine iodide and 1,1'-di-( $\beta$ -carboxy-ethyl)-6,6'-dimethoxy-9-ethyl-benzthio-carbocyanine, for the coupler and/or sensitizer, respectively, used in Example 1 above, so as to obtain an excellent emulsion for the cyan image.

Example 2.—Production of an emulsion for the magenta image

45 The same procedure is adopted as in Example 1, except that the sensitizer there employed is replaced by 30 mg. of 1-( $\beta$ -carboxy-ethyl)-1'-ethyl-6-phenyl-6'-methoxy-benz-thio-pseudocyanine, and the coupler there employed is replaced by 10 g. of 1-phenyl-3-heptadecyl-5-pyrazolone. After coating, exposure, development and so on in the same manner as described in Example 1 a clear intensive magenta is secured. The stability of the finished emulsion prior to coating and the storability of the finished layer are both excellent as in Example 1.

55 Substantially equivalent results may be secured by substituting any of the following couplers, namely 1-phenyl-3-stearoylamo-pyrazolone-5, 1-(2',4'-dichlorophenyl)-3-heneicosyl-pyrazolone-5, 1-(2',4',6',-trichlorophenyl)-3-heptadecylamino-pyrazolone-5 and 1-phenyl-3-heptadecyl-pyrazolone-5, and/or any of the following sensitizers: namely 1-( $\beta$ -carboxy-ethyl)-1'-ethyl-6,6'-dimethoxy-benzseleno-pseudocyanine iodine, 1'-( $\beta$ -carboxy-ethyl)-1'-ethyl-5-methyl-6,6'-dimethoxy-benzseleno pseudocyanine iodide and 1-( $\beta$ -carboxy-ethyl)-1'-ethyl-6-phenyl-6'-methoxy-benzthio-pseudocyanine for the coupler and/or sensitizer, respectively, used in Example 2 above, so as thus to yield an excellent emulsion for the magenta image.

Example 3.—Production of a multi-layer film

70 The emulsion described in Example 1 for the cyan or blue-green image is first coated onto a film base or other support, and then the emulsion described in Example 2 for the magenta image is superimposed upon it. A yellow filter layer which contains colloidal silver or a bleach-

able pigment is then applied, and followed by an unsensitized emulsion layer which contains a dispersed yellow coupler such as for example N-(p-benzoylacetamino-benzenesulphonyl) - N - octadecyl - N - methyl - amine.

If this multi-layer material after exposure is developed in a color developer then, after removal of the silver, a negative color image is obtained. If on the contrary the material after exposure is subjected to the reversal development process, and thus is developed first in, for example, metol-hydroquinone and only afterwards in a color developer then, after removal of the silver, a color positive is obtained. The sensitivity of the material behind green and red-filters is practically the same after storage as in the fresh condition.

*Example 4*

12 grams of 1-(2',4',6'-trichlorophenyl)-3-hepta-decyl-pyrazolone-(5) were dissolved in 40 cc. of hot ethanol, and then 13 cc. of 2 N sodium hydroxide were added and the mixture was diluted with 60 cc. of water at 40° C. The warm solution was admixed with a solution of 10 grams of gelatin and 1.5 grams of sodium dodecylbenzene sulfonate in 100 cc. of water at 40° C. While stirring, the highly viscous gelatin solution was neutralized with 13 cc. of 2 N acetic acid or mineral acid. An extremely fine dispersion was obtained thereby, which dried completely transparent upon pouring. If it is desired to remove the alcohol and salts, the dispersion is allowed to solidify and is washed with water after it has been comminuted. Subsequently the solidified gelatin is melted again and, after admixing it with a silver halide emulsion containing as a green-sensitizer 1-( $\beta$ -carboxyethyl)-1'-ethyl-6,6'-dimethoxybenzene-selenocyanine iodide, it is poured into a film carrier and dried. After exposure and development, a clear purple image is obtained.

*Example 5*

200 cc. of a 6% gelatin solution and 20 cc. of 10% sodium alkyl naphthalene sulfonate were heated in a heatable mixer at 80° C. with a mixture consisting of 6 grams of 1-hydroxy-2-naphthoic acid-octadecylamide (M.P. 78° C.) and of 6 grams of 1-hydroxy-2-naphthoic acid-lauryloxypropylamide (M.P. 42° C.) and dispersed at 18,000 r.p.m. After admixing with a silver halide emulsion containing 1,1-di-( $\beta$ -carboxyethyl)-6,6'-dichloro-9-ethyl-benzene-selenocyanine iodide as a red sensitizer, the procedure of Example 4 was followed to form a clear blue-green image.

Various modifications of the process of the invention may be made without departing from the spirit or scope thereof and it is to be understood that the invention is to be limited only as defined in the appended claims.

We claim:

1. A process for the preparation of color photographic emulsions for the production of the cyan image which comprises forming a silver halide emulsion sensitized with a compound selected from the group consisting of a compound having the formula



wherein R is a lower alkyl radical, R' is selected from the group consisting of hydrogen, lower alkyl radicals, lower alkoxy radicals, naphthylene and halogen, n is an integer from 1 to 2, A is a lower alkylene radical, Y is selected from the group consisting of selenium and sulfur atoms and X is an anion and its betaine derivatives, forming a dispersion of a color coupler selected from the group consisting of phenols and  $\alpha$ -naphthols lacking solubilizing groups and having an aliphatic hydrocarbon residue of

10 to 21 carbon atoms therein in the absence of oil formers and mixing the said silver halide emulsion and the said dispersion to form the desired color photographic emulsions.

5 2. The process of claim 1 wherein the color coupler is selected from the group consisting of 1-hydroxy-4-chloro-2-naphthoic acid N-octadecylamide, 1-hydroxy-2-naphthoic acid N-octadecylamide, 1-hydroxy-2-naphthoic acid N-dodecyloxybutylamide and 1-hydroxy-2-naphthoic acid N-octadecylamide.

10 3. The process of claim 1 wherein the sensitizer is selected from the group consisting of 1,1'-di-( $\beta$ -carboxyethyl)-6,6'-dichloro-9-ethyl-benzene-selenocyanine iodide, 1,1'-di( $\beta$ -carboxyethyl)-5,5'-dimethoxy-9-ethyl-benzene-selenocyanine iodide, 1,1'-di-( $\beta$ -carboxyethyl)-6,6'-dichloro-9-ethyl-benzene-selenocyanine iodide and 1,1'-di-( $\beta$ -carboxyethyl)-6,6'-dimethoxy-9-ethyl-benzene-selenocyanine iodide.

15 4. A process for the preparation of color photographic emulsions for the production of the magenta image which comprises forming a silver halide emulsion sensitized with a compound having the formula



25 30 35 wherein one R1 is a lower alkyl radical and the other R1 is —A—COOH wherein A is a lower alkylene radical, R' is selected from the group consisting of hydrogen, lower alkyl, lower alkoxy, naphthylene and halogen, n is an integer from 1 to 2, Y is selected from the group consisting of selenium and sulfur atoms and X is an anion, forming in the absence of an oil former a dispersion of a pyrazolone color coupler lacking solubilizing groups and having an aliphatic hydrocarbon residue having 10 to 21 carbon atoms and mixing the said silver halide emulsion and the said dispersion to form the desired color photographic emulsions.

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9

a color coupler selected from the group consisting of phenols and  $\alpha$ -naphthols lacking solubilizing groups and having an aliphatic hydrocarbon residue having 10 to 21 carbon atoms and superimposing thereon a silver halide emulsion lacking solution promoters and containing as the sensitizer a compound having the formula



wherein one  $R_1$  is a lower alkyl radical and the other  $R_1$  is  $-A-COOH$  wherein A is a lower alkylene radical,  $R'$  is selected from the group consisting of hydrogen, lower alkyl, lower alkoxy, naphthylene and halogen,  $n$  is an integer from 1 to 2, Y is selected from the group consisting of selenium and sulfur atoms and X is an anion, and a pyrazolone color coupler lacking solubilizing groups and having an aliphatic hydrocarbon residue having 10 to 21 carbon atoms, then a yellow filter layer and finally an unsensitized emulsion layer containing a dispersed yellow coupler.

8. A color photographic emulsion for the production of the cyan image lacking solution promoters comprising a silver halide emulsion containing as the sensitizer a compound selected from the group consisting of a compound having the formula



wherein R is a lower alkyl radical,  $R'$  is selected from

the group consisting of hydrogen, lower alkyl radicals, lower alkoxy radicals, naphthylene and halogen,  $n$  is an integer from 1 to 2, A is a lower alkylene radical, Y is selected from the group consisting of selenium and sulfur atoms and X is an anion and its betaine derivatives and a color coupler selected from the group consisting of phenols and  $\alpha$ -naphthols lacking solubilizing groups and having an aliphatic hydrocarbon residue having 10 to 21 carbon atoms.

9. A color photographic emulsion for the production of the magenta image lacking solution promoters comprising a silver halide emulsion containing as the sensitizer a compound having the formula



wherein one  $R_1$  is a lower alkyl radical and the other  $R_1$  is  $-A-COOH$  wherein A is a lower alkylene radical,  $R'$  is selected from the group consisting of hydrogen, lower alkyl, lower alkoxy, naphthylene, and halogen,  $n$  is an integer from 1 to 2, Y is selected from the group consisting of selenium and sulfur atoms and X is an anion and a pyrazolone color coupler lacking solubilizing groups and having an aliphatic hydrocarbon residue having 10 to 21 carbon atoms.

#### References Cited by the Examiner

##### UNITED STATES PATENTS

- |           |        |               |       |        |
|-----------|--------|---------------|-------|--------|
| 2,640,776 | 6/1953 | Spence et al. | ----- | 96—100 |
| 3,249,360 | 8/1960 | Julian        | ----- | 96—100 |

NORMAN G. TORCHIN, Primary Examiner.

J. T. BROWN, Assistant Examiner.